

## UNITED STATES PATENT OFFICE

ARTHUR S. ROBERTS, OF HENDERSONVILLE, NORTH CAROLINA

## METHOD OF CROSS-DYEING FABRICS

No Drawing. Application filed December 17, 1927, Serial No. 240,921. Renewed December 11, 1930.

My invention relates to a process of dyeing cotton and that type of regenerated cellulose known as xanthate silk or viscose when woven in the same fabric.

An object of my invention is to provide a further combination of certain dyestuffs and chemicals which will act to dye either the cotton or type of regenerated cellulose and leave the other portion of the fabric undyed.

10 Another object of my invention is to provide a process of dyeing fabrics woven from cotton and certain types of regenerated cellulose in which the cotton may be dyed one color and the regenerated cellulose 15 another color.

I have discovered that by using certain dyestuffs which are capable of being developed such as primuline, Schultz No. 616, thiazole yellow 2GM Schultz No. 198, 20 diamine green B, Schultz No. 474 and the like, which are diazotized and subsequently developed with the various developers, such as beta naphthol, resorcin, phenol, naphthalamine ether, developer Z, salicylic acid, and 25 the like, will, when introduced into a dye machine in a manner and at a temperature as set forth in a following paragraph, will act to dye the viscose or xanthate silk portion 30 of the fabric and leave the cotton portion undyed or only slightly stained.

I have also discovered that certain substantive or direct dyes selected from the group consisting of direct yellow S2G Schultz No. 10, direct rubine B, Schultz No. 35 313, direct brilliant blue G, Schultz No. 415 and the like with an addition of approximately ten ounces of sodium hydroxide per each forty gallons of water used, and at a temperature of approximately 120° F. will 40 act to dye the cotton part of the fabric to the shade desired and leave the xanthate silk or viscose portion undyed or only slightly stained.

Although I do not desire to be bound by 45 the explanation which follows, I have found the best method of procedure for the cross-dyeing of xanthate silk or viscose and cotton when woven in the same fabric, with the above named dyes substantially as follows: The cloth is first wet out in cold

water and left in a roll on the dye machine. The machine is filled with water which is heated to approximately 160 degrees Fahrenheit and the dyestuff after having been dissolved in a pail is poured into the machine, one half for the first end or dip and the remaining one half for the second end or dip, after which the goods are given as many ends as is desired, to bring up the shade. This bath is then wasted and the goods

60 slightly rinsed, and the diazotizing bath, composed of approximately twelve ounces of sodium nitrite and forty ounces of hydrochloric acid, together with sufficient water is then run into the machine and the goods

65 worked in this liquor at ordinary room temperature until the coupling process is completed, which ordinarily requires from three to five dips or ends in this bath. This diazotizing bath is then wasted and goods given

70 a thorough washing in cold water. The developing bath composed of the developer for the shade desired together with the sodium hydroxide or hydrochloric acid necessary to dissolve the developer, plus sufficient water

75 is then run into the machine and the cloth is given sufficient runs or ends in this liquor to develop the shade desired. In this connection it is well enough to state, that if a gold color is desired on the viscose, resorcin

80 seven ounces, sodium hydroxide fifteen ounces is used as the developer. If a blue shade is desired, fifteen ounces of naphthalamine ether, seven and one half ounces of hydrochloric acid is used for each forty gallons

85 of water for 100 lbs. of goods. It then can plainly be understood that the other developers are used in the like proportion, beta naphthol for a red and phenol for a yellow shade.

90 After the dies have been developed as to the shade and color desired, the goods are washed with water at approximately 180 degrees Fahrenheit containing soap enough

95 to form a good emulsion for several ends or dips, and then rinsed in cold water slightly acidified with acetic acid to remove any trace of the sodium hydroxide. The above is for the purpose of dyeing the xanthate or viscose portion of the fabric and leaving the

cotton portion undyed or only slightly stained.

The dyebath for the cotton portion of the fabric is then made of one or more of the 5 substantive or direct dyes together with sufficient water at a temperature of approximately 120 degrees Fahrenheit and the goods are given sufficient dips or ends in this liquor to produce the color and shade desired on this part of the fabric, after which 10 this bath is also wasted and the goods given a thorough washing in cold water and are squeezed and dried.

I have also discovered that by combining 15 any of the two above dyebaths, at a temperature of approximately 140 degrees Fahrenheit the color on the xanthate silk or viscose will be diazotized and developed while the substantive or direct dyes will take only 20 on the cotton portion of the fabric. To illustrate—if the primuline and the direct rubine B. conc is made up in the same bath to the approximate amount of four ounces of the former and twelves ounces of the 25 latter, the goods given from three to five ends or dips in this bath at a temperature of approximately 140° Fahrenheit, rinsed, diazotized, and developed with phenol and sodium hydroxide to the amounts given 30 above it will be found after washing the fabric thoroughly that the viscose contains yellow color while the cotton is colored a bluish red. Primuline and direct rubine B. conc in the same bath developed with resorcine and sodium hydroxide would give a gold silk and red cotton. Primuline and direct rubine B. conc developed with naphthamine ether would give a blue silk and a red cotton. while primuline and direct yellow S2G developed with beta naphthol and sodium hydroxide would give a red silk and a yellow cotton.

Thus those skilled in the art to which this process belongs can plainly understand 45 that by combining the two complete dyebaths, diazotizing baths, and developing baths, two separate and distinct colors may be dyed on a combination fabric composed of xanthate silk or viscose and cotton at 50 one and the same operation and time.

In the specification, I have set forth a preferred embodiment of my invention, and although specific terms are employed, they are used in a generic and descriptive sense only, and not for purposes of limitation, the scope of my invention being set forth in the appended claims.

I claim—

1. That method of cross-dyeing a fabric composed of viscose and cotton fibers which comprises subjecting the fabric to a dyebath containing dyes that are capable of being developed selected from the group consisting of Schultz Numbers 616, 198, 474, direct dyestuffs selected from the group con-

sisting of Schultz Numbers 10, 313, and 415 together with sodium hydroxide at a temperature of approximately 140° F. then subjecting the fabric to a bath containing a diazotizing agent at ordinary room temperature, then subjecting the fabric to a bath containing the developing agent, to produce two separate colors on the fabric.

2. That method of cross-dyeing a fabric composed of regenerated cellulose and cotton fibers which comprises subjecting the fabric to a dyebath containing dyes that are capable of being developed selected from the group consisting of Schultz Numbers 616, 198, 474, and the like, direct dyestuffs selected from the group consisting of Schultz Numbers 10, 313, 415 and the like, together with sodium hydroxide at a temperature of approximately 140° F. then subjecting the fabric to a bath containing a diazotizing agent at ordinary room temperature, then washing the fabric in cold water, then subjecting the fabric to a bath containing the developing agent, subsequently washing in cold water, and finally washing in water at a temperature of approximately 180° F. containing a neutral soap solution which acts to dye the viscose portion of the fabrics one color and the cotton portion another color.

In testimony where I affix my signature.  
ARTHUR S. ROBERTS.

9

10

11

11

11

120

120

130